

## UNITED STATES PATENT OFFICE

JENÖ TAUSZ, OF KARLSRUHE, GERMANY

## PROCESS FOR PURIFYING HYDROCARBON OILS

No Drawing. Application filed July 8, 1924, Serial No. 724,792, and in Germany July 16, 1923.

This invention relates to the processes for purifying hydrocarbon oils, such as petroleum, shale oil, brown coal tar oil, pit coal tar oil, and the products obtained therefrom.

5 It is known that hydrocarbon oils which have only been distilled in the manner usual in the art, after some time assume a dark colour and in some cases a disagreeable odour and that there is a formation of resin and 10 a separation of a deposit.

In order to avoid these objectionable phenomena, the oils are, after distillation, subjected to a refining process.

Now I have found that these objectionable 15 phenomena are not caused by the hydrocarbons themselves, but by certain compounds present in these oils and containing besides carbon and hydrogen, also oxygen, nitrogen and sulfur. Such compounds are especially 20 oxygen-containing bodies, such as furane and its homologues, and nitrogen-containing bodies, such as pyrrol and its homologues, and derivatives of these compounds.

In the usual refining processes, for instance 25 when refining the hydrocarbons by treatment with sulfuric acid, not only these objectionable constituents are acted upon and removed, but also the olefines, though there would be no objection to leaving them in the oil. This, 30 of course, causes a loss of valuable material, which loss is especially remarkable in the case of oils containing a large percentage of unsaturated constituents, such oils being obtained for instance by destructive distillation 35 of brown coal or lignite and by the known cracking processes.

Now, I have further found that the constituents, causing the dark coloration or the disagreeable odour or the formation of resins 40 and deposits, have a well defined boiling temperature, depending upon the nature of the oils, and that consequently these constituents can be separated and removed by fractional distillation, if this is very exactly performed.

45 According to my invention, I proceed in contradiction to the distillation processes usual in the treatment of mineral oils. Indeed, in distilling mineral oils, it is now usual to separate the oils into fractions boiling 50 within relatively large limits, while accord-

ing to my invention, the distillation is performed in apparatus allowing of fractions being obtained which distil over within very narrow boiling limits, the fractions being preferably collected separately from degree 55 to degree or even less. Such apparatus are for instance known and used in the art of rectifying alcohol. By applying this method, it is possible, by separately collecting the products which are distilled within such narrow limits, to ascertain first by a preliminary test, which fractions of the material under treatment contain the objectionable constituents, which fractions may be termed resin forming fractions. These fractions are removed when distilling the oils in practice, while the other fractions not containing such constituents may be collected within any convenient limits. It is therefore possible to refine the oils by a simple exact fractional 65 distillation and to avoid partly or wholly the usual refining processes by means of chemical substances and the losses connected therewith. As the boiling points of the resin forming substances depend upon the pressure, it 70 is advisable to keep the pressure constant during the distillation.

In certain cases, especially in the case of oils having a high boiling point, it is advantageous to effect the distillation under reduced 80 pressure, as the boiling points of the resin forming substances are modified by a change of pressure. Thus, it is possible in many cases to prevent other substances which at a certain pressure would be distilled over at 85 the same temperature as the resin forming substances, from being removed together with the latter, the boiling point of such substances being modified in another manner than that of the resin forming substances, if the pressure is changed.

In certain cases it is also possible to apply reduced pressure only during a part of the distillation.

Similar methods can be applied to the further treatment of the separated resin forming fractions.

In certain cases the purification can be obtained more rapidly, by first forming fractions boiling within somewhat larger limits, 100

comprising more than one degree, and then removing the resin forming constituents by subjecting these fractions to a further exact fractional distillation as described.

5 The raw materials can either be immediately treated as described, or first be subjected to a slight preliminary refining treatment as usual in the art of treating petroleum.

10

*Examples*

1. Benzine, obtained by destructive distillation of brown coal and having 0.780 specific gravity, is distilled by means of a rectifying apparatus provided with an efficient dephlegmator, and the distilled products are separately collected from degree to degree. It is found that the fractions distilling over at 62, 86 and 108° C. contain colouring, resin forming and deposit forming constituents, while the other fractions do not contain such substances. It is therefore possible to obtain a pure product, not containing objectionable constituents by simply distilling the said oil 25 and removing the fractions above referred to. Other starting materials can be treated in an analogous manner.

2. When distilling a brown coal benzine having a resin forming fraction boiling at 30 138° C. and containing a remarkable percentage of xylols, most of these xylols is distilled over together with the said resin forming fraction. If, however, the distillation is effected under reduced pressure, for 35 instance a pressure of 100 millimeters of mercury, the boiling point of the resin forming fraction is modified otherwise than that of the xylols. The resin forming substances are under these conditions distilled at 82° C., 40 while the xylols are boiling at 78° C. Thus, by applying reduced pressure it is possible to remove the resin forming substances by a simple but exact fractional distillation, a loss of xylol being avoided.

45 3. In the case referred to in Example 2 it is also possible to perform the distillation first at ordinary pressure, the pressure being kept constant until a temperature of 125° C. is reached, and then to apply reduced pressure. By proceeding in this manner, the boiling point of the resin forming fractions is modified in another manner than that of the hydrocarbons boiling at the same temperature at ordinary pressure, and the same 55 result is obtained as in Example 2.

In a similar manner the resin forming fractions, which have been separated, can be further treated.

What I claim is:—

60 1. The process for purifying hydrocarbon oils, which comprises separating a test portion from the oil, distilling said portion and collecting therefrom fractions within narrow limits to determine the boiling temperatures 65 of fractions forming resins and deposits

and causing coloration and disagreeable odors, then distilling the main body of the oil fractionally and at the ascertained temperatures, and separating such fractions from the remainder of the oil.

2. The process for purifying hydrocarbon oils containing a large percentage of unsaturated hydrocarbons and olefines, which comprises separating a test portion from the oil, distilling said portion and collecting therefrom fractions within narrow limits to determine the boiling temperatures of fractions forming resins and deposits and causing coloration and disagreeable odors, then distilling the main body of the oil fractionally 70 and without substantial loss of olefines and at the ascertained temperatures, and separating such fractions from the remainder of the oil.

75 3. The process for purifying hydrocarbon oils, which comprises separating a test portion from the oil, distilling said portion and collecting therefrom fractions within narrow limits to determine the boiling temperatures of fractions forming resins and deposits and causing coloration and disagreeable odors, then distilling the main body of the oil fractionally 80 and at the ascertained temperatures, and separating such fractions from the remainder of the oil.

85 4. The process for purifying hydrocarbon oils, which comprises separating a test portion from the oil, distilling said portion and collecting therefrom fractions within narrow 90 limits to determine the boiling temperatures of fractions forming resins and deposits and causing coloration and disagreeable odors, then distilling the main body of the oil fractionally and at the ascertained temperatures, and separating and discarding such fractions 95 from the remainder of the oil.

100 5. The process for purifying hydrocarbon oils, which comprises separating a test portion from the oil, distilling said portion and collecting therefrom fractions within narrow 105 limits to determine the boiling temperatures of fractions forming resins and deposits and causing coloration and disagreeable odors, then distilling the main body of the oil fractionally and at the ascertained temperatures, separating such fractions from the remainder of the oil, and completing the fractional distillation of the oil and blending said fractions.

110 5. The process for purifying hydrocarbon oils, which comprises separating a test portion from the oil, distilling said portion and collecting therefrom fractions within narrow 115 limits to determine the boiling temperatures of fractions forming resins and deposits and causing coloration and disagreeable odors, then distilling under constant pressure the main body of the oil fractionally and at the ascertained temperatures, and separating such fractions from the remainder of the oil.

120 6. The process for purifying hydrocarbon oils, which comprises separating a test portion from the oil, distilling said portion and collecting therefrom fractions within narrow 125 limits to determine the boiling temperatures of fractions forming resins and deposits and causing coloration and disagreeable odors, then distilling under reduced constant pressure the main body of the oil fractionally and at the ascertained temperatures, and separating 130

ing such fractions from the remainder of the oil.

7. The process for purifying hydrocarbon oils, which comprises separating a test portion from the oil, distilling said portion and collecting therefrom fractions within narrow limits to determine the boiling temperatures of fractions forming resins and deposits and causing coloration and disagreeable odors, then distilling the main body of the oil fractionally, distilling the separated fractions under reduced constant pressure and at the ascertained temperatures, and separating such fractions from the remainder of the oil.

15 In testimony whereof I have affixed my signature:

JENÖ TAUSZ.

20

25

30

35

40

45

50

55

60

65